

March 19, 1963

R. E. DONALDSON ET AL

3,082,121

FLAMEPROOF CELLULOSE ACETATE FABRICS

Filed April 24, 1961



**Fig. 1**



**Fig. 2**



**Fig. 3**

*Raymond E. Donaldson  
Charles C. White*

INVENTORS

*By R. Frank Smith  
Walter O. Donaldson*

ATTORNEYS

1

3,082,121

FLAMEPROOF CELLULOSE ACETATE FABRICS  
 Raymond E. Donaldson and Charles C. White, Kingsport,  
 Tenn., assignors to Eastman Kodak Company, Rochester,  
 N.Y., a corporation of New Jersey

Filed Apr. 24, 1961, Ser. No. 104,795  
 18 Claims. (Cl. 117—136)

This invention relates to the treatment of carpets produced from cellulose acetate fibers and yarns to give this type of fabric flame-retardant properties.

Heretofore, many treatments of various kinds of fabrics have been proposed for rendering such fabrics resistant to burning. For example, it has been proposed to flameproof or render resistant to burning cotton or viscose fabrics by depositing on such fabric various water soluble salts from their aqueous solutions, but it has been found that these agents are not effective in flameproofing cellulose acetate carpet materials at low add-ons such as 1-3% of the flame-retardant agent based on the weight of the fabric or fiber. When it has been attempted to employ higher add-ons of the order of 5-25%, for example, the so-treated fabric has been found to have an excessively harsh hand or the carpet is stiff and boardy and has a poor appearance. It has also been found that add-ons of this amount of the flame-retardant agent degrades the physical properties of the carpet. Many water soluble materials such as sodium tetraborate, sodium phosphate, ammonium phosphate, ammonium sulfamate, sodium carbonate, potassium bicarbonate, and many others have been proposed for flameproofing cotton and viscose but none of these materials have been found to be effective in flameproofing cellulose acetate carpets.

In addition to the agents referred to above, a number of other inorganic salts have been shown to have some efficacy as flameproofing agents when applied to various textile fibers and fabrics but in the course of the investigative work which led up to the present invention we have not found that any of these materials are effective in flameproofing cellulose acetate carpets at commercially acceptable add-ons, that is, an amount of the agent sufficient to contribute flame-retarding properties but at the same time not give rise to undesirable physical properties such as poor or harsh hand, stiffness or boardiness, or poor appearance of the carpet fibers.

By the terms "flame retardant" or "flameproofing agent" as used herein and in the appended claims, we refer to an agent which will render the fiber or fabric material to which it is applied self extinguishing, that is, not supporting combustion after having been exposed to an open flame for 30 seconds. By the same token, when we refer herein and in the appended claims to a "flame resistant" or "flameproofed" fabric, we refer to a fabric which has this property of being self extinguishing or not supporting combustion after exposure to an open flame for 30 seconds.

This invention accordingly has as an object the flameproofing of fibers and fabrics, particularly those composed of or containing cellulose acetate fibers.

Another object is to provide a means of flameproofing a rug fabric in which the fibers constituting the pile of the rug consist of or contain a high proportion of cellulose acetate fibers.

Another object is to provide a process of flameproofing a rug fabric in which the fibers constituting the pile of the rug consist of or contain a high proportion of cellulose acetate fibers by treating the fabric with an improved and novel flameproofing agent.

Another object is to provide a process of flameproofing a rug construction in which the pile consists of or contains cellulose acetate fibers by an expedient in which

2

the flameproofing agent is incorporated in and held in the backing binder of the rug and available for later deposition on the rug fibers in a simple and effective manner.

Another object is to provide a flameproof or flame-resistant rug fabric in which the fibers constituting the pile of the rug consists of or contains a high proportion of cellulose acetate fibers with a very low add-on of flameproofing agent.

Another object is to provide a means of flameproofing a rug construction in which the pile is composed of cellulose acetate fibers without adversely affecting the hand of the fabric, rendering it stiff and boardy or adversely affecting the appearance of the fibers.

Another object is to provide a means of flameproofing a rug construction in which the pile is composed of cellulose acetate fibers tufted into a jute back which will not adversely affect the cellulose acetate rug fibers and will not cause chemical deterioration of the jute back or the carpet fiber.

Another object is to provide an improved flame-resistant or flameproofed rug construction in which the pile consists of or contains a substantial proportion of fiber of cellulose acetate.

Other objects will appear hereinafter.

These objects are accomplished by the following invention which, in its broader aspects, comprises depositing on or in a rug construction consisting of or containing cellulose acetate fibers a group I alkali metal formate. According to one embodiment of the invention, the carpet is simply treated with an aqueous solution of the alkali metal formate under such conditions that, upon drying of the treated carpet, the alkali metal formate is deposited on the carpet fiber preferably in an amount corresponding to 1-2%, based on the weight of the treated carpet fibers. In this embodiment, for example, a 10-40% solution of an alkali metal formate such as sodium formate, potassium formate or lithium formate may be simply sprayed on the fabric and the water removed by evaporation or drying, leaving a surface deposit of the formate clinging to the fibers. In another embodiment of the invention, the alkali metal formate may be mixed with the latex or other resinous binders commonly employed as the back size coating which locates the pile loops into the base fabric, which is usually jute. The alkali metal formate in this mixture may constitute

from 1 to 25% by weight of total solids of the composition, although we prefer to employ an amount of the formate corresponding to 10 to 14% of the total solids of the back sizing composition. After the back size coating is applied and properly hardened, the rug fabric may then simply be sprayed with water which leaches a portion of the alkali metal formate out of the backing layer and deposits it in the form of a thin film of alkali metal formate solution on the surface of the fibers of the rug.

While the amount of the alkali metal formate thus deposited is not critical it is believed that about 1%, based on the weight of the carpet fibers, is thus deposited. In any event, upon evaporation of the water a deposit of the solid alkali metal formate is left on the fiber surface to produce the desired flame resistant effect. It should be noted at this point that one of the particular features of novelty of our invention is the fact that a carpet flameproofed in accordance therewith may be washed numerous times without losing its flameproof character. This is because the backsize coating in effect provides a reserve of flameproofing agent, namely, the alkali metal formate which may be brought to the surface of the carpet fiber by successive washings.

In the accompanying drawing, FIGURE 1 is an isometric view of a carpet construction treated in accordance with the process of the invention.

FIGURE 2 is a view showing the carpet construction of FIGURE 1 in detail for a small portion of the carpet.

FIGURE 3 is a schematic illustration showing the method of depositing a latex layer containing an alkali metal formate on the back of a carpet construction such as shown in FIGURES 1 and 2.

Referring to FIGURES 1 and 2 the numeral 1 designates a carpet backing fabric which may be a jute fabric, or example, onto which has been tufted cellulose acetate carpet yarns 2 in the manner more specifically illustrated in FIGURE 2. The numeral 3 designates a conduit in the form of a header which supplies an aqueous solution of an alkali metal formate through a plurality of spray nozzles 4 in the form of a spray onto the surface of the tufts or loops 2. After spraying the treated carpet is simply dried in a current of warm air, thus leaving deposited on the tufts or loops of the fabric, particles of solidified alkali metal formate flameproofing agent 5 as shown in FIGURE 2.

Referring to FIGURE 3, the numeral 6 designates a latex back sizing composition which can be conveniently contained in hopper 7 and fed therefrom through delivery orifice 8 in a layer 9 on to the fabric backing 1 of a tufted cellulose acetate or similar synthetic fiber rug construction, the thickness of the deposited layer being determined by the use of a doctor blade or other equivalent device (not shown). In this case the alkali metal formate is held in solution or suspension in the deposited latex layer. The fabric is treated in a current of warm air to solidify the latex backing after which the fabric may be sprayed or otherwise treated with water to leach the alkali metal formate from the latex backing into the tufts of the carpet construction and thereby render it flame-proof.

In the following examples and description we have set forth several of the preferred embodiments of our invention but they are included merely for purposes of illustration and not as a limitation thereof.

#### Example 1

A cellulose acetate carpet is prepared by tufting a cellulose acetate carpet yarn into a jute backing. This carpet is back sized with a commercial latex back sizing formulation having the following composition:

| Parts by weight                                          |     |
|----------------------------------------------------------|-----|
| aqueous solution of styrene-butadiene latex (50% solids) | 100 |
| sulfur                                                   | 2   |
| inc oxide                                                | 5   |
| inc dibutyl dithiocarbamate                              | 3   |
| potassium oleate                                         | 2   |
| lay dispersion (15% solids)                              | 100 |
| i- $\beta$ -naphthyl-p-phenylene diamine                 | 1   |

The back sizing composition is deposited on the back surface of the rug in any convenient manner, as by running the rug underneath a hopper from which the back sizing composition flows at a controlled rate. The thickness of the coating is determined by the application of a doctor blade or a similar device. The deposited coating is cured and vulcanized by passing the coated material through an oven supplied with hot air, the material passing through the oven at a rate predetermined to effect the proper curing and vulcanization of the back sizing.

The carpet face is then sprayed with a 10% solution of sodium formate in water and the treated carpet then dried. Under such circumstances a deposit of 2% of sodium formate, based on the weight of the carpet fiber, is deposited on the carpet. The treated carpet is then conditioned to approximately zero percent humidity and tested by subjecting the carpet to an open flame for 30 seconds. The carpet is found to extinguish itself as soon as the flame is removed, while an untreated control carpet

of the same material and construction subjected to the same test conditions continued to burn.

#### Example 2

A cellulose acetate carpet is prepared as described in Example 1 and treated with an aqueous solution of lithium formate which, on evaporation of the water component, left a deposit of 4%, based on the weight of the carpet fiber, of the formate salt. This carpet treated with lithium formate does not burn and is self-extinguishing after the flame is removed.

A cellulose acetate carpet is prepared as described in Example 1 and is treated as described above with an aqueous dispersion containing as solids 50% colloidal silica and 50% sodium formate in such an amount as to deposit 4% solids on the carpet. The so-treated carpet does not burn, is self-extinguishing and shows the good anti-soiling properties obtained by the use of a colloidal silica.

#### Example 3

A cellulose acetate carpet is prepared by tufting lofted cellulose acetate yarn into a jute backing. A back sizing composition is prepared having the following ingredients:

| Parts by weight                      |      |
|--------------------------------------|------|
| Back sizing composition of Example 1 | 82.7 |
| Sodium formate                       | 14.0 |
| Sodium-N-methyl-N-oleyltaurate       | 3.3  |

This back sizing composition is deposited on the back surface of the rug and cured as described in Example 1. In a separate operation the carpet face is sprayed with water and dried by passing the carpet through a chamber heated by air flowing therethrough at a temperature of 120° C. The dry carpet is found to be flameproofed as measured by the flameproofing test described above.

#### Example 4

A cellulose acetate carpet is prepared by tufting lofted cellulose acetate yarn into a jute backing. A back sizing composition is prepared having the following ingredients:

| Parts by weight                      |      |
|--------------------------------------|------|
| Back sizing composition of Example 1 | 96.0 |
| Potassium formate                    | 1.0  |
| Sodium-N-methyl-N-oleyltaurate       | 3.0  |

This back sizing composition is deposited on the back surface of the rug and cured as described in Example 1. In a separate operation the carpet face is sprayed with water and dried by passing the carpet through a chamber heated by air flowing therethrough at a temperature of 120° C. The dry carpet is found to be flameproofed as measured by the flameproofing test described above.

#### Example 5

A cellulose acetate carpet is prepared by tufting lofted cellulose acetate yarn into a jute backing. A back sizing composition is prepared having the following ingredients:

| Parts by weight                      |      |
|--------------------------------------|------|
| Back sizing composition of Example 1 | 87.0 |
| Lithium formate                      | 10.0 |
| Sodium-N-methyl-N-oleyltaurate       | 3.0  |

This back sizing composition is deposited on the back surface of the rug and cured as described in Example 1. In a separate operation the carpet face is sprayed with water and dried by passing the carpet through a chamber heated by air flowing therethrough at a temperature of 120° C. The dry carpet is found to be flameproofed as measured by the flameproofing test described above.

#### Example 6

A cellulose acetate carpet is prepared by tufting lofted cellulose acetate yarn into a jute backing. A back sizing composition is prepared having the following ingredients:

| Parts by weight                      |      |
|--------------------------------------|------|
| Back sizing composition of Example 1 | 87.0 |
| Lithium formate                      | 10.0 |
| Sodium-N-methyl-N-oleyltaurate       | 3.0  |

This back sizing composition is deposited on the back surface of the rug and cured as described in Example 1. In a separate operation the carpet face is sprayed with water and dried by passing the carpet through a chamber heated by air flowing therethrough at a temperature of 120° C. The dry carpet is found to be flameproofed as measured by the flameproofing test described above.

#### Example 7

A carpet prepared as in Example 4 is subjected to a cleaning scour such as is customarily employed in com-

mercial rug cleaning plants. This is done by applying a foaming cleaner such as the product sold under the trade name "Artloom Carpet Shampoo," which is a concentrated aqueous detergent or soap solution, to the fiber surface of the carpet and thereafter scrubbing with brushes. The scoured carpet is allowed to dry. Upon bringing a sample of the treated carpet material to zero humidity and testing for flammability, it is found that the material does not burn and is self-extinguishing when the initiating flame is removed, while a carpet of the same material and construction, but lacking the flameproofing formate in the back sizing coating, continues to burn. The scouring operation in this case brings up the formate flameproofing agent and deposits it on the surface of the fibers in the manner described above. This process may be repeated many times and the carpet still will retain its flameproof characteristics due to the leaching of the alkali metal formate onto the fibers each time the carpet is wet by water.

*Example 8*

A cellulose acetate carpet is prepared as described in the first two paragraphs of Example 1. The carpet face is then sprayed with a 20% solution of potassium formate in water and the treated carpet then dried. Under these conditions a deposit of 2% of potassium formate, based on the weight of the carpet fiber, is deposited on the carpet. Upon applying the flameproofing test described above the carpet is found to extinguish itself as soon as the flame is removed, while an untreated carpet of the same material and construction subjected to the same testing conditions continued to burn.

In the above examples and in the appended claims we have referred to a latex back sizing composition. By the term latex we include both natural and synthetic latices, including natural rubber latex, styrene-butadiene copolymers, neoprene, and latices of the acrylic type such as the commercially available polyacrylates, the poly(vinyl)-chlorides and similar polymeric flexible film-forming materials. It is also to be understood that the latex back sizing composition may contain, as indicated above, various fillers such as titanium dioxide, clays, sulfur, curing accelerators, oxidation inhibitors, and other such materials commonly used in the art.

As will be evident from the above examples and description, our invention has many unexpected and outstanding advantages over the flameproofing practices of the prior art. For example, cellulose acetate carpets may now be flameproofed by the application of very low add-ons of the flameproofing material, an especial advantage flowing from this fact being that the cellulose acetate carpet may be flameproofed without the production of boardiness or stiffness of the fabric and without other degradation of the physical properties of the acetate yarn or the backing fabric employed in the carpet construction. Our invention also makes possible the flameproofing of cellulose acetate carpets at an extremely low cost as compared to that involved in the customary methods of flameproofing other fabrics. In this connection it should be particularly pointed out that the flameproofing of cellulose acetate carpet constructions has been impractical or impossible until the advent of the present invention. Thus we have solved a peculiar and long existing problem in the cellulose acetate carpet field. It should also be noted that in that form of our invention in which the flameproofing formate salt is employed as a component of the back sizing composition, there is provided an effective reservoir of the flameproofing agent which may be brought up onto the fibers as desired by the normal washing or scouring process or by simply wetting the carpet construction and subsequently allowing it to dry. To the best of our knowledge and belief this is an entirely unique method of obtaining the flameproofing of cellulose acetate carpets.

Although the invention has been described in considerable detail with particular reference to certain pre-

ferred embodiments thereof, variations and modifications can be effected within the spirit and scope of the invention as described hereinabove, and as defined in the appended claims.

5 We claim:

1. A flameproof cellulose acetate carpet in which cellulose acetate fibers are tufted into a backing fabric, said fibers containing on their surface as the flameproofing agent an alkali metal formate.

10 2. The carpet of claim 1 in which the flameproofing agent is sodium formate.

3. The carpet of claim 1 in which the flameproofing agent is potassium formate.

15 4. The carpet of claim 1 in which the flameproofing agent is lithium formate.

5. The process of flameproofing a carpet composed of cellulose acetate fibers tufted into a carpet fabric backing which comprises applying to the rug fibers an aqueous solution of an alkali metal formate and thereafter removing

20 the water from the applied solution to leave on the fibers a deposit of the formate.

6. The process of claim 5 in which the solution is 1 to 10% aqueous solution of an alkali metal formate.

7. The process of claim 5 in which the aqueous solution is 1 to 30% of an alkali metal formate and the water is removed by drying the rug at a temperature below 180° C.

8. The process of claim 5 in which the flameproofing agent is sodium formate.

30 9. The process of claim 5 in which the flameproofing agent is potassium formate.

10. The process of claim 5 in which the flameproofing agent is lithium formate.

11. A flameproof cellulose acetate carpet in which cellulose acetate fibers are tufted into a carpet fabric backing and back sized with a latex back sizing composition containing as a flameproofing agent an alkali metal formate.

12. A flameproof cellulose acetate carpet in which cellulose acetate fibers are tufted into a carpet fabric backing and back sized with a latex back sizing composition containing as a flameproofing agent 1 to 25%, based on the weight of the total solids of the back size composition, of an alkali metal formate.

13. The carpet of claim 12 in which the alkali metal formate is sodium formate.

14. The carpet of claim 12 in which the alkali metal formate is potassium formate.

15. The carpet of claim 12 in which the alkali metal formate is lithium formate.

16. A flameproof cellulose acetate carpet in which cellulose acetate fibers are tufted into a carpet fabric backing and back sized with a latex back sizing composition containing as a flameproofing agent 10 to 14%, based on the weight of the total solids of the back size composition, of an alkali metal formate.

17. The process of flameproofing a cellulose acetate carpet in which cellulose acetate fibers are tufted into a carpet backing fabric and back sized with a latex back sizing composition containing 1 to 25%, based on weight of the total solids of the composition, of an alkali metal formate, which comprises wetting the carpet with water whereby to leach a portion of the alkali metal formate from the back sizing composition and draw it up and deposit it on the surface of the cellulose acetate fibers.

18. The process of flameproofing a cellulose acetate carpet in which cellulose acetate fibers are tufted into a carpet backing fabric and back sized with a latex back sizing composition containing 10 to 14%, based on weight of the total solids of the composition, of an alkali metal formate, which comprises wetting the carpet with water whereby to leach a portion of the alkali metal formate from the back sizing composition and draw it up and deposit it on the surface of the cellulose acetate fibers.